

## UNITED STATES PATENT OFFICE

IRVING C. HONEGGER, OF HOUSTON, TEXAS, ASSIGNOR TO ALUMINUM COMPANY OF AMERICA, OF PITTSBURGH, PENNSYLVANIA, A CORPORATION OF PENNSYLVANIA

## PROCESS OF ATTACHING METAL FOIL TO A SURFACE

No Drawing.

Application filed May 12, 1931. Serial No. 538,957.

This invention relates to the coating of articles with metal foil, and especially to processes of attaching foil to the article to be coated.

5 Metal foil possesses various advantages as a coating for articles of widely diverse character and use. One advantage is due to the flexibility of metal foil, which permits its intimate application to irregular surfaces, in corners, and the like; for example, in covering shingles, pavements, containers, and other objects. Metal foils generally possess a bright surface, so that they have heat reflecting properties which render such coatings valuable for certain purposes. Aluminum foil is particularly desirable for these purposes, and, in addition to the properties generally possessed by metal foil, its high thermal expansivity adapts it as a covering

10 for articles which are subject to expansion and contraction. Also, aluminum foil is resistant to weathering and other chemical influences, such as acids.

Prior to my invention, no practical means

15 had been available for satisfactorily attaching metal foil to the wide variety of materials of varying composition and surface character which it is desired to coat. The general practice in attaching a material in

20 sheet form to another article is to use liquid adhesives, which, for various reasons, are undesirable and unsuited for the purpose. Their proper use requires skilled judgment in deciding when the adhesive has assumed

25 the proper consistency, or adhesiveness, after being applied to the foil, and the quality of coating therefore depends upon a personal element. There is also the danger in using such adhesives that air pockets will be trapped under the foil, thus reducing the efficacy

30 of the coating.

Further objections to such prior procedures arise from the necessity for using such liquid adhesives where the coating operation is effected, and this is particularly disadvantage-

ous in field operations. In all such procedures, involving manual application of the adhesive, non-uniform application of the adhesive generally results, with uneconomical consequences. Also, where heated adhesives

50 are used there is the constant danger of injury to the operators. More serious objections, however, are due to the lightness and flexibility of the foil, which make its handling difficult. Thus, air currents tend to cause wrinkling as it is applied, so that it is not easy to obtain smooth and tightly adherent coating. Especially is this true in outdoor work when wind is blowing, under

55 which conditions the foil may be torn easily.

60 All of these factors have militated against successful foil coating prior to this invention.

It is among the objects of this invention to provide a process of coating surfaces with metal foil which is simple, applicable to the coating of a great variety of surfaces, effective under widely differing conditions, economical, does not require cumbersome apparatus or skilled manipulation, and overcomes many of the disadvantages of prior methods of coating with metal foil.

This invention is predicated on my discovery that these and other objects are accomplished by applying a layer of asphalt to one side of a sheet of foil, drying or congealing the film, and then pressing the coated side directly against the surface to be covered by applying heat and pressure through the foil.

In the preferred embodiment of the invention foil is prepared for use by passing it over a roller running in molten asphalt, to apply a layer of asphalt to one side of the foil. The asphalt film is cooled quickly to congeal it, and the thus-coated foil is coiled, or otherwise packaged, and kept in this condition until needed.

In the use of this material the foil is placed with the asphalt film directly against a surface to be foiled, whether of wood, glass,

metal, composition, concrete or other material, and heat and pressure are applied through the foil. Under the influence of the heat the asphalt is softened, and the pressure applied to the foil forces it into intimate contact with the surface being coated. The asphalt flows into the surface irregularities, and upon again cooling good adhesion results. The heat and pressure may be applied simultaneously by any suitable means, for instance by a hot smoothing iron or roller.

In the preferred embodiment of the invention bright aluminum foil is used. The asphalt coating may be thin, the thickness being, of course, dependent upon the character of the surface to be coated. For example, rough surfaces usually require heavier coatings than do smooth surfaces. The thinness of the foil and its high heat conductivity insure rapid softening of the asphalt coating, permitting it to be pressed readily into contact with the surface, so that the laying operation is rapid. Because of its especially high thermal conductivity, aluminum foil is particularly efficacious from this standpoint. In addition to its property of congealing and being softened under heat, which permits preparation of the coated foil away from its field of use, asphalt is desirable as a binder because it wets and adheres to surfaces differing widely in character. The method thus provided is advantageous also because it minimizes the hazard of air pockets, which are commonly encountered in applying coatings with liquid adhesives. Such air pockets tend to cause peeling, and to weaken the coating.

A particular advantage of the invention results from congealing of the asphalt coating. This stiffens the foil and makes it much more convenient to handle under widely varying conditions than foil not so provided with a hardened asphalt coating. For instance, the foil does not tend to wrinkle when applied to the surface to be coated, so that it is easier to obtain unwrinkled tight coatings of satisfactory quality than where the foil is not coated, or where liquid adhesives are used. Particularly, it makes the foil more amenable to use for outdoor coating operations, and reduces damage through tearing.

Both the asphalt and the foil repel water, so that these coatings are useful in preventing passage of water through the coated article. This quality may be useful, for example, in conserving moisture, as in curing concrete; and this property is enhanced by the heat-reducing properties of the foil, particularly bright aluminum foil, which tend to lower the temperature of the object beneath it. Moreover, under extremes of temperature the asphalt film possesses sufficient plasticity for the foil to adjust itself without buckling or cracking, as in contraction

and expansion of tanks or pavements. And on expansion of the underlying structure, as on swelling of wood, there is sufficient elasticity to afford adjustment of both the asphalt film and the metal foil without damaging the coating. A further advantage of this coating is that over long periods of time the attaching asphalt, even though only a film, retains its valuable qualities.

Further advantages of the invention are that the foil may be prepared for use and stored until needed, without deterioration of the adhesive. This reduces the equipment needed at the place of use, and particularly the human element is reduced greatly, because the necessity for judging as to the proper condition of adhesive when applying coating is dispensed with, it being necessary only to apply enough heat and pressure to cause the desired adherence. Moreover, economies result from the uniformity of the asphalt coating obtained by mechanical application, and the danger of operators being burned by hot adhesives is minimized.

According to the provisions of the patent statutes, I have explained the principle of my invention, and have described what I now consider to represent its best embodiment. However, I desire to have it understood that, within the scope of the appended claims, the invention may be practiced otherwise than as specifically described.

I claim:

1. The process of attaching metal foil to a surface, comprising applying a layer of asphalt to one side of a sheet of foil, congealing said layer to harden it and stiffen the foil, placing the coated side of the stiffened foil in direct contact with a surface to be covered by said foil, and applying heat and pressure through the foil to soften and press said coating into adherent contact with said surface.

2. The process of attaching aluminum foil to a surface, comprising applying a layer of asphalt to one side of a sheet of aluminum foil, congealing said layer to harden it and stiffen the foil, placing the coated side of the stiffened foil in direct contact with said surface, and applying heat and pressure through the foil to soften and press said coating into adherent contact with said surface.

3. The process of attaching aluminum foil to a surface, comprising applying a layer of liquefied asphalt to one side of a sheet of aluminum foil, congealing said layer to harden it and stiffen the foil, placing the coated side of the stiffened foil in direct contact with said surface, applying a heated metallic presser element to the exposed surface of the foil to soften said asphalt and press it into intimate contact with the surface to cause adherence of the foil thereto.

4. The process of attaching aluminum foil to a substantially rigid surface, comprising

- applying a layer of asphalt to one side of a sheet of aluminum foil, congealing said layer to harden it and stiffen the foil, placing the coated side of the stiffened foil in direct contact with said substantially rigid surface, and applying heat and pressure through the foil to soften said asphalt and press it into adherent contact with said surface to cause adherence of the foil thereto.
- 5 10 5. As a new article of manufacture for coating surfaces, aluminum foil with a layer of asphalt congealed on one side thereof, whereby the foil is stiffened.

15 In testimony whereof, I sign my name.  
IRVING C. HONEGGER.

20

25

30

35

40

45

50

55

60

65